

H. P. BOSTAPH.

## PROCESS OF OBTAINING COKE AND BY-PRODUCTS FROM COAL.

APPLICATION FILED JAN. 19, 1916.

1,204,647.

Patented Nov. 14, 1916.

2 SHEETS—SHEET 1.



**WITNESSES:**

WITNESSES.

F. T. Chapman

BY

E. G. Siggars.

*Attorney*

H. P. BOSTAPH.

PROCESS OF OBTAINING COKE AND BY-PRODUCTS FROM COAL.

APPLICATION FILED JAN. 19, 1916.

1,204,647.

Patented Nov. 14, 1916.

2 SHEETS—SHEET 2.



WITNESSES:

Howard D. Orr.

F. T. Chapman.

Harvey P. Bostaph, INVENTOR,

BY

*E. G. Siggars.*

Attorney

# UNITED STATES PATENT OFFICE.

HARVEY P. BOSTAPH, OF DETROIT, MICHIGAN.

## PROCESS OF OBTAINING COKE AND BY-PRODUCTS FROM COAL.

1,204,647.

Specification of Letters Patent.

Patented Nov. 14, 1916.

Application filed January 19, 1916. Serial No. 73,012.

To all whom it may concern:

Be it known that I, HARVEY P. BOSTAPH, a citizen of the United States, residing at Detroit, in the county of Wayne and State 5 of Michigan, have invented a new and useful Process of Obtaining Coke and By-Products from Coal, of which the following is a specification.

This invention has reference to a process 10 of obtaining coke and by products from coal, and its object is to produce coke containing such a percentage of volatile matter as to provide a smokeless fuel burning freely with a long flame, and also to produce condensable by-products of superior quality and of increased quantity.

In accordance with the present invention the coal, by which term it is meant to include both the substance ordinarily known as 20 coal and other carbonaceous materials suitable for the purposes of the present invention, is subjected in relatively thin masses to a comparatively low, but gradually increasing temperature, in a manner to cause 25 the distillation to progressively proceed from one long edge of each thin mass of coal toward the other long edge, at which latter point the gases of distillation have free escape. Such escape of the gases is facilitated 30 by subjecting the coal during the coking process to subatmospheric conditions, whereby the temperature employed in the distilling operation may be sufficiently low to prevent any harmful effect upon the volatilized 35 products.

The coal during the process of coking, and while under subatmospheric pressure, is first subjected to a temperature of about 700° F., which temperature is finally increased to 40 about 1000° or 1100° F., in accordance with the coal being treated, although with some coals the maximum temperature may be as low as about 900° F. Since the coal is first heated at the exterior or peripheral portion, 45 distillation and coking begin at such peripheral portion and the coked material acts as a heat insulator requiring the raising of the temperature to an injurious or undesirable degree if the distillation and coking is to 50 proceed solely by heat conducted through the previously coked portions. But by

dividing the coal into relatively thin bodies or masses separated by webs of material of heat conducting qualities superior to the coke, the heat is conducted by the webs past 55 the sides of the coked portions at the periphery and acts progressively along the sides of the thin masses of coal. The distillation and coking therefore proceeds uniformly toward that edge of each thin mass of coal 60 remote from the edge first affected by the heat without any necessity of unduly heating the outer edge or peripheral portion of the subdivided mass of coal. Tapering each thin mass of coal from the outer toward the 65 inner edge contributes to this end for the mass to be heated decreases in proportion to the distance from the periphery. Such progressive distillation not only insures the 70 final uniform heating of the whole mass by 75 distributing the heat by conduction but prevents the sealing or trapping within the mass of any of the volatile products for the latter are always provided with a ready avenue of escape toward and through the inner 80 or thin edges of the coal masses.

As the coking progresses the escaping volatile products are never forced to pass through coked portions of the mass or a portion of the mass which is at a higher temperature than that at which the volatile products are evolved.

In the practice of the present invention, and because of the treatment of the coal in thin masses, the coking is not only thorough, 85 but is performed within a commercially reasonable time ranging from three hours to four and one-half hours, more or less, the time depending upon the particular grade of coal employed. Furthermore, the subatmospheric condition to which the coal is subjected is continued during the procedures, whereby the condensable by-products of distillation are recovered.

The invention will be best understood 95 from a consideration of the following detailed description, taken in connection with the accompanying drawings forming part of this specification, with the understanding, however, that while the drawings disclose a 100 form of apparatus capable of practising the invention, the latter may be practised with

other apparatus, wherefore the invention in its practice is not confined to any strict conformity with the showing of the drawings, but may be changed and modified in various ways so long as such changes and modifications mark no departure from the salient features of the invention as expressed in the accompanying claims.

In the drawings:—Figures 1 and 1<sup>a</sup> show partly in elevation, partly in section, and partly schematically an apparatus with which the present invention may be practised. Fig. 2 is a view partly in elevation and partly in section showing the core of the retort of Fig. 1 lowered. Fig. 3 is a cross-section of the core on the line 3—3 of Fig. 1.

Before describing the process, and in order to facilitate the description thereof, the structures shown in the drawings will first be described.

There is shown a columnar form shell 1 upright in the installed position and tapering from the bottom toward the top, such shell constituting the body portion of a retort particularly adapted to the practice of the present invention, and which retort is described in detail and claimed in another application Serial No. 73,011 filed on even date herewith for a retort for the destructive distillation of coal.

The shell 1 is provided with an upper head 2 and a lower head 3 having means, which need not be specifically described, for fastening the heads tightly in place to seal them hermetically to the ends of the retort, but in such manner that they may be readily removed as needed. In the particular showing of the drawings the shell 1 has brackets 4 at the lower end supporting the retort upon channel beams 5 forming part of a suitable installation, since in practising the invention on a commercial scale a battery of retorts is provided and suitable supporting structures are arranged for the accommodation of the retorts. Each retort is surrounded by a wall 6 of fire brick spaced a short distance, say, in the neighborhood of two inches, from the shell 1. The wall 6 constitutes a heat equalizing envelop for the retort and is heated by any suitable means, as, for instance, by hot products of combustion which may be applied to the whole battery of retorts at once. While it is not customary to direct flames against the wall or envelop 6, the drawing shows burners 7 with their flames directed toward the wall 6 merely as a ready indication of the fact that the wall or envelop is being subjected to the action of heat of sufficient intensity for the purpose.

Mounted upon the upper face of the head 3, as by supports 8, is a core 9 comprising in the particular showing of the drawing a frusto-conical bottom plate 10, from which

rises a tubular duct 11 having webs 12 radiating therefrom toward the inner wall of the shell into close relation thereto. The core 9 tapers in conformity with the taper of the retort shell 1.

The core 9 when in the retort divides the interior of the latter into a circular series of chambers 13 constituting coal tubes extending longitudinally of the retort and grouped in circular series about the duct 11, with which latter each chamber 13 communicates along its inner long edge by way of numerous perforations 14. With the webs 12 radial, the coal tubes 13 are of segmental form having the widest end at the retort shell and the chambers are of such dimensions that their greatest width measured circumferentially of the retort does not exceed about four inches, and may with advantage be even less than four inches. With a commercial form of retort about nine feet long, the core is about seven feet in length having a diameter at the upper end of about twenty-three inches and at the bottom of about twenty-seven inches. The walls of the retort are approximately one inch in thickness, while the walls of the duct 10 and the webs 12 are approximately three-fourths of an inch in thickness. In a retort of such particular size the coal tubes at their greatest circumferential width are a little less than four inches, say, about three and nine-sixteenths inches, and have a radial depth varying from about six inches at the upper end to about eight inches at the lower end. These dimensions it will be understood have to do with a commercial form of the retort which has been tried and found to give excellent results, but the practice of the invention is not necessarily confined to a retort of the particular dimensions given.

In the practice of the invention the core 9 is lowered from the retort from time to time for the discharge of its contents, and in order to accomplish this, suitable mechanism is provided, the drawings showing in simplified construction a means for the purpose. A suitable framework 15 serves as a guide for a supporting frame 16 having a post 17 thereon in position to engage and carry the head 3. The frame 16 is in turn carried by ropes or cables 17 running over pulleys 18 and provided with counterweights 19 so arranged as to overbalance the carrier 16 and the core 9, but these counterweights are themselves overbalanced when the core contains a charge of coal or coke. Under the last-named conditions, and when the head 3 is released from the retort, the weight of the core with the charge of coke causes the core to lower, raising the counterweights 19, such lowering being controlled by any suitable brake or retarding means not shown in the drawings. The slanting bottom 10

of the core provides an unstable support for the columns of coke off of which they readily slide when freed from the restraint of the shell 1, as when the core is in the lowered position shown in Fig. 2. Since there is a liability of the hot coke, because of its expansion, sticking to the core, or even to the inner walls of the retort, the latter is entered by a steam pipe 20, where-  
 10 by the charge within the retort may be cooled down somewhat before the core is lowered, thus causing a sufficient contraction of the coke to loosen it from adherence to the walls inclosing it, and consequently  
 15 the coke readily gravitates from the core when the latter is lowered from the retort.

The duct 11 opens at the upper end into a chamber 21 in the upper end of the retort, from which chamber there leads a pipe 22 including a controlling valve 23 and connected to another pipe 24, which latter may be common to a battery of retorts and constitutes a vapor line discharging into another pipe 25 on one side of a release valve  
 25 26 therein. The pipe 25 is connected through a valve 27 into a tar tank 28. Leading from the tar tank is a pipe 29 discharging into a condenser drum 30. The pipe 29 includes a tar extractor 31 and a  
 30 vacuum gage 32, and has connected thereto an equalizing valve 33, which, however, need not be described in detail. Leading from the condenser drum 30 is a pipe 34 connected to one end of a condensing coil  
 35 35 having associated therewith a cooling water spray pipe 36. That end of the condensing coil 35 remote from the pipe 34 is connected by a pipe 37 to a washer 38 discharging into a separating tank 39. Leading  
 40 from the separating tank is a pipe 40 communicating with a vacuum pump 41, and the latter discharges into a scrubber 42, from which there leads a pipe 43 to a suitable gasometer, not shown.

45 A water pump 44 supplies water to the separating tank and to the scrubber, and suitable means are provided for supplying water to the washer. An oil pump 45 collects the condensed liquids from the various  
 50 parts of the system and discharges through the pipe 46 to a suitable point of storage.

In the practice of the present invention the coal in relatively thin columns is subjected to the action of heat directed first against one edge, that is, with the retort shown, the outer or peripheral edge, of each column of coal with the heat increasing in intensity from a minimum temperature to a maximum temperature. The heating progresses from the edge first affected toward the opposite edge, particularly along the sides of the coal column, since the walls of the coal tube have greater heat conductivity than the coal itself and especially than  
 60 coked portions of the coal. While the heat-

ing and consequent distillation is progressing through the mass of coal subatmospheric conditions are established by suction apparatus, such as a vacuum pump, so that the volatile matters driven off from the coal  
 70 are withdrawn therefrom as rapidly as formed and through the inner edge of each column of coal.

The external surface of the retort is maintained at about the maximum temperature  
 75 employed, while the core after discharging the coke by being withdrawn from the retort becomes reduced in temperature, so that when a fresh charge of coal is introduced into the retort it is subjected at first to a  
 80 considerably reduced temperature.

With the present invention the maximum temperature need not exceed about 1100° F. and then the temperature of the interior of the retort after discharging the coke and on  
 85 the return of the core thereinto will be in the neighborhood of 700° F., so that the thin mass of coal in each coal tube is subjected to distillation first along the outer edge with the distillation progressing toward the inner edge, and the heat to which the coal is subjected correspondingly increasing toward the maximum temperature  
 90 employed.

Experience has shown that the coking is  
 95 progressive without choking back or trapping the products of distillation when the greatest width of the column of coal does not exceed about four inches and the coking is performed under subatmospheric conditions whereby the volatile products of distillation are withdrawn as rapidly as formed from that edge of the coal column remote from the edge to which the heat is initially applied. Under such circumstances the distillation is completed in from three to four  
 100 and one-half hours, and hence is commercially economical. Furthermore, the treatment of a thin mass of coal in the manner stated and under the conditions named produces a coke containing a sufficient percentage, say, about ten per cent., of the entire volatile matter originally contained in the coal, the product being a smokeless fuel  
 105 burning freely with a long flame, while the amount of volatile matter driven off and recoverable is increased over other coking procedures and is of superior quality because the temperature employed is insufficient to have any harmful effect upon such by-  
 110 products.

Cannel coals treated by the process of the present invention produce a smokeless fuel  
 115 burning with a long flame and useful for steam as well as cupola purposes. The quantity of oils obtained from the cannel coal ranges from two to two and one-half times as much as that obtained from bituminous coal, and the oils are somewhat more highly  
 120 saturated with acids. The coke has a some-  
 130

what similar appearance to wood charcoal but is much firmer and cleaner. The evolved gases, being quickly carried away through the numerous small openings distributed along each coal tube, say, at distances of about six inches from each other, are not burned, and hence when treated by a series of condensers, extractors, washing apparatus and cooling coils, all of which apparatus together with the retort is subjected during the entire process to a relatively high vacuum, the character of the recovered by-products is markedly superior. Because of the treatment of the coal to gradually increasing temperatures within about the limits stated, unusually large quantities of light oils and gases are obtained. The entirely different natures of the oils and acids obtained by the present process from those obtained at higher temperatures is attributed to the fact that the temperatures are not allowed to become excessive. The coke produced retains all the fixed carbon which the coal originally carried.

As an example of the actual practice of the invention certain cannel coals treated showed by analysis:—moisture 2.20, vol. matter 47.35, carbon 42.15, ash 8.30, sulfur 1.30.

An analysis of the coke showed:—volatile matter 11.27, fixed carbon 74.44, ash 14.29, sulfur 1.31.

Out of 1200 pounds of coal there were obtained 854 pounds of coke and 33 gallons of crude oil condensates of dark brown color, with a specific gravity of .995 at 15.5 degrees C., and flowing freely at 27° C.

What is claimed is:—

1. The process of producing coke from coal which consists in subjecting a relatively thin body or mass of coal to the action of heat applied initially at one edge of the mass, maintaining the heat at that edge and applying heat progressively along each side of the mass from one edge to the other, whereby the entire heat for the distillation of the mass does not have to be transmitted through the mass which is adjacent to the edge at which the heat is initially applied.

2. The process of producing coke from coal, which consists in subjecting a relatively thin body or mass of coal to the action of heat applied initially at one edge of the body of coal and progressively along each side thereof, and causing the gases of distillation to escape from the other thin edge of said body of coal.

3. The process of producing coke from coal, which consists in subjecting a relatively thin body of coal to distilling heat applied to one thin edge of the coal and withdrawing the gases of distillation by suction from the other thin edge of the body of coal.

4. The process of producing coke from

coal, which consists in subjecting a relatively thin body of coal to distilling heat applied to one thin edge of the coal, causing the heating to progress along the sides of the body of coal, and withdrawing the gases of distillation by suction from the other thin edge of the body of coal.

5. The process of producing coke from coal, which consists in subjecting the coal in relatively thin masses having the greatest thickness not exceeding about four inches to the action of distilling heat directed against one edge of the mass of coal and withdrawing the products of combustion by suction from the opposite edge of the mass of coal.

6. The method of producing coke from coal, which consists in subjecting the coal arranged in a series of relatively thin masses in close side by side association to the action of distilling heat applied initially and continuously at one long edge of each mass and progressively along each side of each mass toward the other long edge thereof.

7. The method of producing coke from coal, which consists in subjecting the coal arranged in a series of relatively thin masses in close side by side association to the action of distilling heat applied initially and continuously at one long edge of each mass and progressively along each side of each mass toward the other long edge thereof, and removing the products of distillation by suction from the second-named long edges of the masses of coal as rapidly as such products are formed.

8. The process of producing coke from coal, which consists in subjecting a group of relatively thin masses of coal arranged about a central duct to the action of distilling heat directed against the outer long edges of the masses and withdrawing the gases of distillation from the inner long edges through the central duct by suction as rapidly as the gases are formed.

9. The process of producing coke from coal, which consists in subjecting a group of relatively thin masses of coal arranged about a central duct to the action of distilling heat directed against the outer long edges of the masses, conducting the heat along the sides of the thin masses of coal progressively, and in withdrawing the gases of distillation from the inner long edges through the central duct by suction as rapidly as the gases are formed.

10. The process of producing coke from coal, which consists in subjecting the coal in relatively thin masses to the action of distilling heat applied initially at one edge of each mass, maintaining the heat at that edge and applying heat progressively along the sides of each mass toward the other edge thereof, the heat increasing progressively from about 700° F. to about 1000 or 1100°

F., and at the same time withdrawing the gases of distillation as formed by suction from that edge of each mass of coal opposite to the edge at which the heat is initially applied, the maximum temperature employed being varied in accordance with the kind of coal treated.

In testimony, that I claim the foregoing as my own, I have hereto affixed my signature in the presence of two witnesses.

HARVEY P. BOSTAPH.

Witnesses:

J. B. Goss,  
FLORENCE JACOBI.